

## 1

3,008,888

 METHOD FOR THE PRODUCTION OF  
PROCESSED PAPERS

Shigenobu Fujimoto, Tsurumi-ku, Yokohama-shi, Japan  
(38 Ogura, Kawasaki-shi, Kanagawa-ken, Japan)  
No Drawing. Filed June 27, 1958, Ser. No. 744,939  
Claims priority, application Japan July 4, 1957  
2 Claims. (Cl. 204—165)

This invention relates to methods of processing paper and pulp sheets. More particularly, it relates to a method of producing processed paper in which paper made of cellulose of wood such as red pine (*Pinus densiflora*), beech (*Fagus sieboldii*), yezo spruce (*Picea jezoensis*) and Japanese spruce (*Abies sachalinensis*) as well as Japanese paper is treated with sulfuric acid thereby producing processed paper which is much improved in water-resistance and feel and also in strength and especially in tensile strength, tearing strength and bursting strength.

It is known that parchment paper is produced by treating paper with sulfuric acid. Though water-resistant and transparent, parchment paper has defects and is easy to break by bending or tension. Further, known sulfuric acid treatment is not applicable to paper made of cellulose of wood such as red pine, beech and yezo spruce, since it requires a long time to amyloidize uniformly the surface of such paper, and the paper treated with sulfuric acid for a long time is of no practical use due to the fact that amyloid is deposited deep into the paper thereby deteriorating its strength.

Accordingly, an object of the invention is to provide an effective method for processing paper made of said wood fibres and pulp sheet and Japanese paper, in which the surface of the paper is treated uniformly with sulfuric acid for a very short time to obtain a paper improved in water-resistance, feel and strength.

In accordance with this invention, amyloidation of cellulose with sulfuric acid is effected uniformly in a limited layer at the surface of the paper thereby to produce paper having not only a soft feel but also improved characteristics as particularly regards tensile strength, tearing strength, bursting strength and water-resistance. In some cases, the air-permeability is also improved. The present invention thus provides processed paper most suitable for use as packing or bag paper for cement and other powder, as well as for sliding-doors and wall-paper.

The present invention is characterized in that the treatment of paper with sulfuric acid is carried out by passing paper between metal plates to which the superposed medium waves and short waves are applied. These su-

## 2

alkali, or a solution of sodium carbonate or trisodium phosphate may be used.

The superposed waves used in the invention are formed in such a way that each of said electric waves is oscillated separately through, for example, a Colpitts' push-pull circuit and these circuits are joined into a circuit which is connected to the electrodes. If the angular frequencies of the alternating currents thus oscillated are respectively indicated as  $\omega_1$  and  $\omega_2$ , the circuit will have an alternating voltage of the following equation:

$$e_s = \sqrt{2E_1} \sin \omega_1 t + \sqrt{2E_2} \omega_2 t$$

This is not a modulated wave but a voltage in the superposed form of alternating currents  $\omega_1 + \omega_2$  which is termed herein as the superposed wave.

The following examples are given as illustrations of specific embodiments of this invention.

## Example 1

20 Three vats containing sulfuric acid, alkali solution and water respectively are arranged in alignment so that paper to be treated may be passed successively through these vats. The first vat contains sulfuric acid of 55° Bé. and the second alkali vat contains a solution of trisodium phosphate of 13° Bé. In each vat there are provided two metal plates between which the paper is passed. Although sulphuric acid is a conductor, it has sufficient resistance to avoid short-circuiting the plates. The two plates are connected respectively to two specific current generators provided separately to which medium wave of about 800—1000 kc. and short wave of about 25—30 mc. are applied.

25 The currents to be supplied by the two generators are from about 300 milliamperes to 2 amperes and preferably about 1 ampere, respectively. The amounts of currents of the two generators are preferably the same although they may differ to some extent from each other. The superposed currents flowing in the bath exhibit an excellent effect on the paper under treatment giving good water-resistance, strength and feel. After the waves are applied to each bath for about 30 minutes, a paper made from red pine is passed between said metal plates. When the paper is passed through the sulfuric acid bath in 13 seconds, the treatment time of about 26 seconds is sufficient to accomplish the process including water-washing. The paper thus treated has a much improved feel and water-resistance.

30 The following table shows that the strength and elongation of the treated paper is remarkably improved over the untreated paper.

|                            | Bursting Strength (kg.) | Strength ratio | Tensile Strength (kg.) |               | Breaking Length (km.) |       | Elongation (percent) |              |
|----------------------------|-------------------------|----------------|------------------------|---------------|-----------------------|-------|----------------------|--------------|
|                            |                         |                | leng.                  | eros.         | leng.                 | eros. | leng.                | eros.        |
| Known process:             |                         |                |                        |               |                       |       |                      |              |
| Air-dried                  | 8.40                    | 4.32           | 13.03<br>6.01          | 10.80<br>4.49 | 4.98                  | 4.04  | 6.4<br>7.8           | 6.6<br>10.3  |
| Dipped in water for 10 min |                         |                |                        |               |                       |       |                      |              |
| Process of the Invention:  | 8.91                    | 5.24           | 16.9<br>6.84           | 14<br>4.83    | 5.2                   | 4.35  | 6.8<br>8.4           | 7.2<br>13.24 |
| Air-dried                  |                         |                |                        |               |                       |       |                      |              |
| Dipped in water for 10 min |                         |                |                        |               |                       |       |                      |              |

## Example 2

perposed waves may be employed advantageously for alkali treatment and water-washing.

For the alkali treatment, a dilute solution of caustic

Kraft paper was treated in similar manner as in Example 1.

The test results of the paper thus treated were as follows:

|                                                    | Kraft<br>paper<br>untreated | Treated kraft<br>paper |      | 10 |
|----------------------------------------------------|-----------------------------|------------------------|------|----|
|                                                    |                             | A                      | B    |    |
| Tensile strength (Normal) (Kg./15 mm. wide):       |                             |                        |      |    |
| length.....                                        | 6.1                         | 13.1                   | 12.7 |    |
| crossw.....                                        | 2.6                         | 7.5                    | 8.8  |    |
| Tensile strength (Wet) (Kg./15 mm. wide):          |                             |                        |      |    |
| length.....                                        | 0.43                        | 6.2                    | 7.0  |    |
| crossw.....                                        | 0.11                        | 4.0                    | 5.1  |    |
| Bursting strength (Normal) (Kg./cm. <sup>2</sup> ) | 1.6                         | 4.4                    | 4.9  |    |
| Bursting strength (Wet) (Kg./cm. <sup>2</sup> )    | 0.1 and<br>less             | 3.4                    | 3.0  |    |

The above was measured according to JIS P 8113 and P 8112.

Temperature at the time of measurement was 30° C. and the humidity 75% R.H.

The strength in wet condition was similarly measured after dipping in water at 30° C. for 30 minutes.

As described above, the processing of paper according to the invention is effected in a very short time, causing no fear of lowering the strength of the paper but bringing on improvements in strength. Furthermore, this process can be carried out with high efficiency by continuous operation.

The foregoing examples illustrate treatment with sul-

furic acid and alkali phosphate, but it is apparent to those skilled in the art that to said treating liquor there may be added penetrants and buffer agents or, in some cases, dyestuffs, and that an after-treatment with softener such as glycerine may be added.

What is claimed is:

1. In a method for processing paper by passing it successively through a concentrated sulfuric acid bath, a neutralizing bath containing alkaline compound and a water bath, the improvements comprising the steps of spacing two metallic plates to form a path therebetween for said paper in said sulfuric acid bath and simultaneously passing between said metallic plates electric currents, one current having a frequency of from 800 to 1000 kc. and the other current having a frequency of from 25 to 30 mc., so that two currents of different frequencies will be superposed.

2. The improvement as claimed in claim 1, wherein the bath of sulfuric acid is maintained at about 50° Bé. and the alkali bath is a bath of trisodium phosphate at about 13° Bé.

#### References Cited in the file of this patent

#### UNITED STATES PATENTS

|           |          |                |
|-----------|----------|----------------|
| 1,590,595 | Hill     | June 29, 1926  |
| 1,791,248 | Schwartz | Feb. 3, 1931   |
| 2,089,966 | Kassner  | Aug. 17, 1937  |
| 2,852,452 | Hausner  | Sept. 16, 1958 |